# EUROPEAN PATENT APPLICATION

(11) **EP 4 431 077 A1**
(43) Date of publication of application: **18.09.2024**
(21) Application number: 24163475.7
(22) Date of filing: 14.03.2024
(51) Int. Cl.: A61J 1/03, B32B 7/04, B32B 15/04, B65D 75/36, C09J 7/28, C09J 7/35

(54) **BASE BODY FOR A BLISTER CONTAINER AND RESPECTIVE BLISTER COMPONENT FOR PACKAGING PRODUCTS**

(30) Priority: 14.03.2023 IT 202300004821
(71) Applicant: Carcano Antonio S.p.A., 23826 Mandello Del Lario (LC) (IT)
(72) Inventor: GUIDI, Annalisa, 23826 Mandello del Lario (IT); BUSI, Andrea, 23826 Mandello del Lario (LC) (IT)
(74) Representative: Feltrinelli, Secondo Andrea

(57) **Abstract**

The present invention relates to a base body for a blister container as well as to a blister container for packaging products, in particular pharmaceutical products, comprising such base body.

Furthermore, the present invention even relates to a method for obtaining a blister container as above-mentioned.

## Description

### TECHNICAL FIELD OF THE INVENTION

The present invention concerns a base body for a blister container as well as a blister container for packaging products, in particular pharmaceutical products, comprising such a base body.

Furthermore, the present invention also concerns a method of obtaining a blister container as mentioned above.

### STATE OF THE PRIOR ART

The state of the prior art proposes various base bodies that can be used for the production of blister containers as well as respective blister containers, for example of the type "push-through", "peel-off", if desired "easy-peel", "peel-push" or "tear-open".

Typically, the base body of such blister containers is made using a multilayer structure comprising a main layer of thermoplastic material, for example polyvinyl chloride (PVC), which is particularly economical compared to the use of other materials. The cavities or pockets for housing products, in particular pharmaceutical products, are often formed by hot forming and subsequently sealed by the application of a covering film, generally also comprising a multi-layer structure having a main layer of aluminium.

From a functional point of view, by pressing on the back of a housing cavity or pocket defined on the base body, the latter is deformed and the product contained therein is extracted from the container by piercing (in the case of "push-through" blister containers) or by tearing (in the case of "peel-off' blister containers) the covering film.

However, the use of polyvinyl chloride (PVC) as the material of the main layer of the base body is not able to provide an absolute or in any case optimal barrier to gas, humidity and light.

Subsequently, blister containers were designed and manufactured with a base body comprising a multilayer structure with a main layer of aluminum capable of ensuring an optimal barrier to gas, humidity and light. The base body of these blister containers is generally obtained by cold forming and includes, in addition to the main aluminum layer, also at least one external layer, i.e. designed to come into contact with the environment, made of a first plastic material, for example of oriented polyamide (oPA) as well as at least one internal layer, i.e. designed to come into contact with the product to be contained, made of a second plastic material, for example of polyvinyl chloride (PVC). These layers of plastic material are necessary as they ensure adequate mechanical resistance and good cold formability of the base body.

The multilayer structure of the base body of the aforementioned blister containers, i.e. for example oPA/Alu/PVC, poses particular problems from the point of view of sustainability, as the presence of plastic layers considerably complicates the process of disposal and/or recycling of the latter, actually increasing the overall environmental impact of such blister containers.

Furthermore, it should be considered that all the layers of this multilayer structure are, in general, laminated with adhesive, which further increases the complexity in the separation of the layers during disposal and/or recycling.

In this regard, a multilayer structure with a metallic material and one or more plastic materials, for example a configuration of the oPA/Alu/PVC type, requires a complicated, if not impossible, separation process between the metallic material and the one or more plastic materials during disposal and/or recycling.

For a long time, moreover, the current regulations relating to the essential requirements for packaging and packaging waste have proposed, as a general guideline for the creation of more sustainable packaging, the use of single-material structures with minimization of plastic components or, in any case, where it is not possible to opt for a single-material structure, the use of structures that facilitate the separation of the different materials.

It is therefore advantageous and necessary to design and manufacture a base body for a blister container and a respective blister container which make it possible to overcome the above-mentioned disadvantages of the prior art.

### OBJECTS OF THE INVENTION

The technical task of the present invention is therefore to improve the state of the art in the field of blister containers for packaging of products, in particular pharmaceutical products.

An object of the present invention is to provide a blister container and, in particular, a base body for a blister container with performances from the point of view of gas, moisture and light barrier, mechanical resistance and cold formability comparable to those blister containers described in the prior art but exploiting a single-layer or single-material structure and suitable coatings.

Another object of the present invention is to design and manufacture a blister container and, in particular, a base body for a blister container that is more sustainable and, therefore, has a lower environmental impact compared to the blister containers provided by the prior art.

Another object of the present invention is to provide a blister container capable of ensuring optimal extraction of the product, in particular of the pharmaceutical product, from the blister container itself.

A further object of the present invention is to develop a blister container and, in particular, a base body for a blister container which allows a simpler and faster disposal and/or recycling process compared to the blister containers provided by the state of the prior art.

This task and these objects are achieved by a base body for a blister container according to claim 1.

This task and these objects are also achieved by a blister container according to claim 12 as well as by a method of obtaining a blister container according to claim 20.

The dependent claims refer to preferred and advantageous embodiments of the invention.

### BRIEF DESCRIPTION OF THE DRAWINGS

Other characteristics and advantages of the invention will be more evident from the description of an embodiment of a base body for a blister container and a respective blister container, illustrated for indicative purposes in the attached drawings in which:
- figure 1 is a perspective view of a base body for a blister container according to an embodiment of the present invention,
- figure 2 is a cross-sectional view taken along the line A-A of the base body for a blister container according to the embodiment of figure 1,
- figure 3 is a perspective view of a blister container according to an embodiment of the present invention,
- figure 4 is a cross-sectional view taken along the line A-A of the blister container according to the embodiment of figure 3.

In the attached drawings, identical parts or components are identified by the same reference numbers.

### EMBODIMENTS OF THE INVENTION

With reference to the attached figures, the number 1 indicates as a whole a base body for a blister container according to a non-limiting embodiment of the present invention.

The base body 1 according to the present invention can advantageously be used for the production of blister containers of the *"push-through", "peel-off', "easy-peel", "peel-push"* or *"tear-open"* type.

The base body 1 for a blister container according to the present invention defines one or more pockets or cavities 2 designed to contain products, in particular pharmaceutical products, for example lozenges, tablets, capsules, optionally soft capsules, pills, powders, vials, syringes, liquids, gels or similar.

The base body 1 according to the present invention is obtained by cold forming.

The use of cold forming allows to exploit, as will be better seen below, a very thick barrier layer which allows complete or in any case optimal insulation from gas, humidity and light, thereby making it possible an extension of the shelf life of the products to be contained.

Furthermore, the cold forming process avoids heating of the base body 1 and, therefore, saves energy compared to using hot forming.

From a structural point of view, the base body 1 according to the present invention includes a barrier layer 3 made of aluminum which defines a first surface 3a and a second surface 3b opposite to the first surface 3a.

In particular, the barrier layer 3 is coated with:
- a heat-sealing lacquer or varnish layer 4 applied on the second surface 3b and designed to ensure heat-sealing of the base body 1 to a film for covering the one or more pockets or cavities 2 of the base body 1, the heat-sealing lacquer or varnish layer 4 being made wholly or in part, for example for at least 60% or 70%, if desired for at least 80% or 90%, of an elastomeric synthetic resin or a polystyrene-butadiene resin or an acrylic resin or a polymer synthetic resin or a resin of PVC-free polymeric mixtures or an olefin resin or an ethylene resin or an olefin-acrylic resin or an epoxy resin or a methacrylate-based resin or a mixture of two or more of the above resins, and
- a forming aid lacquer or varnish layer 5 applied on the first surface 3a and designed, in use, to come into contact with the external environment, the forming aid lacquer or varnish layer 5 being made wholly or in part, for example for at least 60% or 70%, if desired for at least 80% or 90%, of a crosslinked polyester resin or an epoxy resin or a polystyrene-butadiene resin or an acrylic resin or a synthetic polymer resin or a resin of PVC-free polymeric mixtures or an olefin resin or an ethylene resin or an olefinic-acrylic resin or a methacrylate-based resin or a mixture of two or more resins of the above resins,

As can be understood, the layer of heat-sealing lacquer or varnish 4 is used for subsequent sealing of the base body 1 with a covering film so as to thus obtain a blister container for packaging products while the forming aid lacquer or varnish layer 5 is used to promote and facilitate the cold forming of the base body 1.

In fact, in order to be cold formed, the barrier layer 3 made of aluminum must be covered with a layer of lacquer or forming aid varnish 5 in order to avoid or in any case reduce the possibility of breakages during the forming process of the same.

The base body 1 can be formed with any suitable polygonal plan configuration, for example rectangular, if desired with rounded corners, square or circular, elliptical or the like.

The dimensions of the base body 1 can be set both as a function of the number of pockets or cavities 2 and as a function of the pitch between them, i.e. as a function of the distance between a pocket or cavity 2 or row of pockets or cavities 2 and another previous or subsequent pocket or cavity 2 or previous or subsequent row of pockets or cavity 2.

The one or more pockets or cavities 2 defined on the base body 1 can be present in any suitable number, for example one, two, six, ten and so on, and can be arranged in one or more rows, if desired parallel.

The one or more pockets or cavities 2 can be formed according to the configuration of the product or products to be contained, for example an elongated ellipsoidal configuration in the case of products having a longitudinal dimension that predominates with respect to the transversal dimension, or a substantially spherical configuration in the case of products having a substantially circular plan configuration. The depth of the one or more pockets or cavities 2 can also be set according to the height or thickness of the product(s) to be contained.

Preferably, the thickness of the barrier layer 3 is between 45 µm and 100 µm, preferably between 60 µm and 85 µm or, more particularly, between 70 µm and 75 µm, for example about 72.5 µm.

The aluminum of the barrier layer 3 is advantageously in the form of an aluminum alloy, preferably an alloy belonging to the 1000 or 3000 series of alloys, for example alloy 3105, or to the 8000 series, for example alloy 8011 or alloy 8013.

Optionally, the barrier layer 3 is aluminum in a soft state, for example annealed or soft-tempered aluminum.

More in detail, the barrier layer 3 is preferably subjected to dynamic cooking, that is, during the manufacturing of the base body 1. The coil of the barrier layer 3 is unwound and heated in a suitable oven in order to obtain improved mechanical characteristics and more uniform than static cooking, which involves internal heating of the coil without unwinding the barrier layer 3.

Alternatively, the barrier layer 3 is, in sequence, hot-rolled reaching for example a thickness of 6 mm, roughed up to a thickness of 2 mm, subjected to intermediate annealing, roughened up to a thickness of 0.5 mm, subjected to final rolling and then to final annealing.

In this respect, the aluminum grains of the barrier layer 3 have:
- the average length of the grain between 1 and 20 µm, if desired among 5 and 15, for example between 8 and 10 µm or equal to about 9 µm, and/or
- the average width of the grain between 1 and 20 µm, if desired among 5 and 15, for example between 7 and 9 µm or equal to about 8 µm, and/or
- number of grains for mm² among 5000 and 15000, for example between 8000 and 10000 or equal to about 9100, 9200, 9300, 9400 or 9500, and/or
- size of the grain ASTM between G 5,0 and G 20,0, for example between G 8,0 and G 12,0, if desired among G 9,0 and G 11,0 or equal to about G 10,1, G 10,2, G 10,3, G 10,4 or G 10,5.

As regards the heat-sealing lacquer or varnish layer 4, preferably, the elastomeric synthetic resin is a solvent-based or water-based elastomeric synthetic resin.

Advantageously, the solvent is selected from the group composed of ethyl acetate, cyclohexane, methyl ethyl ketone, dibasic methyl ethyl ketone ester or water.

If desired, the dry residue of the heat-sealing lacquer can be between 5% and 35% by weight of the total weight thereof, for example equal to approximately 20%.

Preferably, the heat-sealing lacquer or varnish layer 4 does not comprise polyvinyl chloride (PVC) and/or does not comprise nitrocellulose.

Optionally, the layer of heat-sealing lacquer or varnish 4 has a grammage of between 0.5 g/m² and 8 g/m², preferably between 1 g/m² and 5 g/m², preferably about 3.5 g/m².

Preferably, the thickness of the heat-sealing lacquer or varnish layer 4 is between 1 µm and 10 µm, for example between about 3.5 µm and about 6 µm.

However, as regards the layer of forming aid lacquer or varnish layer 5, the cross-linked polyester resin is preferably free of bisphenol A.

As it is known, bisphenol A is a substance widely used in combination with other chemical substances for the production of resins and plastics for food use, potentially harmful to health if present in doses exceeding a certain quantity.

Optionally, the forming aid lacquer or varnish layer 5 has a grammage of between 1 g/m² and 8 g/m², preferably between 3 g/m² and 6 g/m², for example approximately 4.5 g/m².

Advantageously, the thickness of the forming aid lacquer or varnish layer 5 is between 1 µm and 10 µm, for example between about 3.5 µm and about 6.5 µm.

The polyester chemical nature can be advantageously selected as it is a chemical nature flexible depending on the molecules to be used, which effectively allows the base body 1 to be cold formed, avoiding breakages.

If desired, the base body 1 also includes at least one layer of silicone oil suitable for food contact on the heat-sealing lacquer or varnish layer 4 and/or on the forming aid lacquer or varnish layer 5, for example with a grammage between 0.2 g/m² and 1 g/m², if desired approximately 0.6 g/m².

Preferably, the thickness of the or each layer of silicone oil is between 0.1 µm and 0.5 µm, for example about 0.3 µm.

Advantageously, the base body 1 also includes at least one layer of slip material, such as for example waxes, on the heat-sealing lacquer or varnish layer 4 and/or on the forming aid lacquer or varnish layer 5.

The slip material gives a slipperiness of between 45 and 100 g, preferably between 60 and 70 g.

Alternatively, according to another non-limiting embodiment of the present invention, the forming aid lacquer or varnish layer 5 could be made entirely or partially of an epoxy resin.

As can be understood, the subject-matter of the present invention is also a blister container 6 for packaging of products, in particular pharmaceutical products, for example lozenges, tablets, capsules, if desired soft capsules, pills, powders, vials, syringes, liquids, gels or similar.

The blister container 6 according to the present invention comprises a base body 1 according to the present invention or according to non-limiting embodiments of the present invention, and a covering film 7 bonded by heat sealing to the layer of heat-sealing lacquer or varnish layer 4 of the base body 1, so as to close the one or more pockets or cavities 2 of the base body 1.

Preferably, the covering film 7 includes a first layer 8 made of aluminum which defines a first face 8a and a second face 8b opposite to the first face 8a as well as a second layer 9 applied on the second face 8b and designed to ensure heat sealing with the heat-sealing lacquer or varnish layer 4, the second layer 9 being or comprising a heat-sealing lacquer or varnish.

According to the non-limiting embodiment of the present invention shown in figures 3 and 4, the heat-sealing lacquer or paint of the second layer 9 has the same composition as the heat-sealing lacquer or varnish layer4.

Advantageously, the thickness of the first layer 8 is between 10 µm and 60 µm, for example between about 20 µm and about 35 µm.

Preferably, the thickness of the second layer 9 is between 1 µm and 10 µm, for example between about 3.5 µm and about 6 µm.

Advantageously, the first layer 8 is raw or hard tempered aluminum or semi-raw or semi-hard tempered aluminium, for example in the H24, H26 or H48 state.

According to the non-limiting embodiment of the present invention shown in figures 3 and 4, the first layer 8 is coated with a layer of primer 10 applied on the first face 8a designed to facilitate the printing of written and/or graphic information.

Advantageously, the primer layer 10 does not comprise polyvinyl chloride (PVC) and/or does not comprise nitrocellulose.

Optionally, the primer layer 10 is polyester based.

Preferably, the thickness of the primer layer 10 is between 0.1 µm and 2 µm, for example about 1 µm.

According to the non-limiting embodiment of the present invention shown in figures 3 and 4, the covering film 7 consists of the first layer 8 coated with the second layer 9 on the second face 8b, and with the primer layer 10 on the first face 8a.

According to another non-limiting embodiment of the present invention (not shown in the figures), the covering film 7 consists of the first layer 8 coated with the second layer 9 on the second face 8b, and with the primer layer 10 on the first face 8a, the primer layer 10 having a print layer applied thereon.

According to a further non-limiting embodiment of the present invention (not shown in the figures), the covering film 7 consists of the first layer 8 coated with the second layer 9 on the second face 8b, and with the primer layer 10 on the first face 8a, a printing layer applied on the primer layer 10 and a protection layer, for example a protective varnish or lacquer, applied on the printing layer.

Preferably, the blister container 6 includes a percentage by weight of aluminum on the total weight of the same greater than 90%, for example equal to about 92.5%, if desired equal to about 95% of its weight.

It should be noted that the presence of respective lacquers or paints on the first surface 3a and on the second surface 3b of the barrier layer 3 of the base body 1 and the presence of a lacquer or paint on the second face 8b of the first layer 8 of the covering film 7 allows the disposal and/or recycling of the blister container 6 as if it were a mono-material of aluminium, effectively allowing 100% disposal and/or recycling, thus increasing its sustainability and environmental impact.

Subject-matter of the present invention is also a method of obtaining a blister container, according to the present invention or according to non-limiting embodiments of the present invention, for the packaging of products, in particular pharmaceutical products.

The method according to the present invention initially includes the step of providing a base body 1.

It should be noted that, as already described above, the base body 1 is obtained by cold forming and, thus, the base body 1 provided in the method is a cold formed base body 1.

The step of providing a covering film 7 is then envisaged.

Finally, the step of heat-sealing the layer of heat-sealing lacquer or varnish layer 4 and the covering film 7 to obtain the blister container 6 is included.

Preferably, the method comprises, before the cold forming of the base body 1, the step of spreading or applying a layer of silicone oil suitable for food contact on the layer of heat-sealing lacquer or varnish layer 4 and/or on the forming aid lacquer or varnish layer 5, for example with a grammage between 0.2 g/m² and 1 g/m², preferably around 0.6 g/m².

Advantageously, the heat sealing step occurs at a temperature between approximately 140°C and approximately 260°C.

The base body 1 as well as the blister container 6 provide performances from the point of view of the gas, humidity and light barrier, mechanical resistance and cold formability comparable to the blister containers described in the prior art, however exploiting a single structure layer or single material and appropriate coatings.

In particular, the base body 1 as well as the blister container 6 guarantee excellent barrier properties to gas, humidity and light, also allowing the conservation of special drugs, for example anti-tumor drugs, which require particular storage conditions.

Furthermore, one should consider that in the case of storing special drugs, some machines insufflate nitrogen to maintain an inert atmosphere and, thanks to the present invention, a guarantee that the nitrogen does not escape from the blister container 6 is obtained.

Furthermore, the base body 1 as well as the blister container 6 provide an alternative, innovative and more sustainable solution with a lower environmental impact compared to the blister containers described in the prior art.

In this regard, the base body and the respective blister container 6 described in the present discussion allow to obtain a simpler and faster disposal and/or recycling process compared to the blister containers provided by the prior art.

It has thus been seen that the invention fully achieves the proposed objects.

Modifications and variations of the invention are possible within the scope defined by the claims.

## Claims

1. Base body (1) for a blister container, defining one or more pockets or cavities (2) designed to contain products, in particular pharmaceutical products, obtained by cold forming, said base body (1) comprising:
- a barrier layer (3) made of aluminum which defines a first surface (3a) and a second surface (3b) opposite to said first surface (3a),
- a heat-sealing lacquer or varnish layer (4) applied on said second surface (3b) and designed to ensure heat-sealing of said base body (1) to a film for covering said one or more pockets or cavities (2) of said base body (1), said heat-sealing lacquer or varnish layer (4) being made wholly or in part of an elastomeric synthetic resin or a polystyrene-butadiene resin or an acrylic resin or a polymer synthetic resin or a resin of PVC-free polymeric mixtures or an olefin resin or an ethylene resin or an olefin-acrylic resin or an epoxy resin or a methacrylate-based resin or a mixture of two or more of the above resins, and
- a forming aid lacquer or varnish layer (5) applied on said first surface (3a) and designed, in use, to come into contact with the external environment, said forming aid lacquer or varnish layer (5) being made wholly or in part of a crosslinked polyester resin or an epoxy resin or a polystyrene-butadiene resin or an acrylic resin or a synthetic polymer resin or a resin of PVC-free polymeric mixtures or an olefin resin or an ethylene resin or an olefinic-acrylic resin or a methacrylate-based resin or a mixture of two or more resins of the above resins,
wherein the aluminum of said barrier layer (3) is in the form of an aluminum alloy belonging to the 1000, 3000 or 8000 alloy series.
wherein the aluminum grains of the barrier layer (3) have:
- the average length of the grain between 1 and 20 µm,
- the average width of the grain between 1 and 20 µm.

2. Base body (1) according to the previous claim, wherein the aluminum grains of the barrier layer (3) have:
- the average length of the grain between 5 and 15 µm,
- the average width of the grain between 5 and 15 µm.

3. Base body (1) according to claim 1 or 2, wherein said elastomeric synthetic resin is a solvent-based or water-based elastomeric synthetic resin.

4. Base body (1) according to the preceding claim, wherein said solvent is selected from the group consisting of ethyl acetate, cyclohexane, methylethylketone, methylethylketone-dibasic ester.

5. Base body (1) according to any one of the preceding claims, wherein said heat-sealing lacquer or varnish layer (4) does not comprise polyvinylchloride or PVC.

6. Base body (1) according to any one of the preceding claims, wherein said heat-sealing lacquer or varnish layer (4) does not comprise nitrocellulose.

7. Base body (1) according to any one of the preceding claims, wherein the dry residue of said heat-sealing lacquer or varnish layer (4) is comprised between 5% and 35% by weight of the total weight thereof.

8. Base body (1) according to any one of the preceding claims, wherein said crosslinked polyester resin is free of bisphenol A.

9. Base body (1) according to any one of the preceding claims, wherein the thickness of said barrier layer (3) is between 45 µm and 100 µm.

10. Base body (1) according to any one of the preceding claims, wherein the thickness of said heat-sealing lacquer or varnish layer (4) is between 1 µm and 10 µm or between about 3.5 µm and about 6 µm.

11. Base body (1) according to any one of the preceding claims, wherein the thickness of said forming aid lacquer or varnish layer (5) is between 1 µm and 10 µm or between about 3.5 µm and about 6.5 µm.

12. Base body according to any of the previous claims, comprising at least one layer of material slipping on the heat-sealing lacquer or varnish layer (4) and/or on the forming aid lacquer or varnish layer (5), said slipping material conferring a slipperiness between 45 and 100 g.

13. Blister container (6) for packaging products, in particular pharmaceutical products, comprising a base body (1) according to any one of the preceding claims, and a covering film (7) constrained by heat sealing to the heat-sealing lacquer or varnish layer (4) of said base body (1), so as to close said one or more pockets or cavities (2) of said base body (1).

14. Blister container (6) according to the preceding claim, wherein said covering film (7) comprises a first layer (8) made of aluminum which defines a first face (8a) and a second face (8b) opposite to said first face (8a) as well as a second layer (9) applied on said second face (8b) and designed to guarantee heat-sealing with said heat-sealing lacquer or varnish layer (4), said second layer (9) being or comprising a heat-sealing lacquer or varnish.

15. Blister container (6) according to the preceding claim, wherein the heat-sealing lacquer or varnish of said second layer (9) has the same composition of said heat-sealing lacquer or varnish layer (4).

16. Blister container (6) according to claim 14 or 15, wherein the thickness of said first layer (8) is between 10 µm and 60 µm or between about 20 µm and about 35 µm.

17. Blister container (6) according to any one of claims 14 to 16, wherein the thickness of said second layer (9) is between 1 µm and 10 µm or between about 3.5 µm and about 6 µm.

18. Blister container (6) according to any one of claims 14 to 17, wherein said first layer (8) is coated with a primer layer (10), applied to said first face (8a), aimed at facilitating the printing of written and/or graphic information.

19. Blister container (6) according to the preceding claim, wherein said primer layer (10) does not comprise polyvinyl chloride or PVC and/or does not comprise nitrocellulose.

20. Blister container (6) according to any one of claims from 14 to 19, comprising a percentage by weight of aluminum on the total weight of the same greater than 90%.

21. Method for obtaining a blister container (6) according to any one of claims 13 to 20 for packaging products, in particular pharmaceutical products, comprising the steps of:
- providing said base body (1),
- providing said covering film (7),
- heat-sealing said heat-sealing lacquer or varnish layer (4) and said covering film (7) to obtain said blister container (6).

22. Method according to the preceding claim, comprising, before cold forming of said base body (1), the step of spreading or applying a silicone oil layer suitable for food contact on said heat-sealing lacquer or varnish layer (4) and/or on said forming aid lacquer or varnish layer (5).

23. Method according to claim 21 or 22, wherein said heat-sealing step takes place at a temperature comprised between about 140°C to about 260°C.
